

# UNITED STATES PATENT OFFICE.

WALTER F. PRINCE, OF ELIZABETH, NEW JERSEY.

## METHOD FOR REMOVING SULFUR FROM CAST-IRON.

1,081,403.

Specification of Letters Patent.

Patented Dec. 16, 1913.

No Drawing.

Application filed May 8, 1912. Serial No. 696,019.

*To all whom it may concern:*

Be it known that I, WALTER F. PRINCE, a citizen of the United States, residing at Elizabeth, county of Union, and State of

5 New Jersey, have invented certain new and useful Improvements in Methods for Removing Sulfur from Cast-Iron, of which the following is a full, clear, and exact description.

My invention pertains to the removal of 10 sulfur from cast iron.

It is a matter of common knowledge that 15 sulfur is one of the most detrimental elements in making cast iron that is met with in the foundry. Ordinary pig iron is roughly estimated to contain the following amounts: in number one pig, .03; in number two pig, about .04 or .05; in number three pig, .06 and so on. When this iron is graded it is sold as to its grade, and the price varies with the varying amount of sulfur which it contains. When this iron containing say, .04, goes into the cupola and is melted it picks up more sulfur from the fuel in the cupola and issues therefrom containing about .07, .08 and as high as .1.

This is especially true when mineral fuel is used, as it is difficult to prevent the metal from taking up sulfur. It is well known also that excess of sulfur in cast iron develops a multiplicity of micro-sulfur flaws therein and when this excessive amount of sulfur is present the cast iron presents a honey-combed appearance. The deleterious effects of these treacherous sulfur areas, as well as other microscopic flaws, with their prolonged ramifications spreading along the ultimate crystals of the metal and thereby destroying metallic cohesion, is a matter that is of grave consequence. Constant vibration

40 ultimately loosens the metallic adherence of the crystals of the metal, especially in areas where these micro-flaws of sulfur exist. Cankering by internal corrosion and disintegration is induced whenever the terminations of the sulfid areas or other flaws

45 in any way become exposed at the surface of the metal, either to the action of atmospheric or other oxidizing influences. In many other ways it can also be observed how injurious these sulfid flaws are in cast iron.

At present about 60% of good castings are obtained to the amount of iron melted. Consequently 40% of the castings has to go back to the cupola each day which has picked up enough sulfur to make this scrap carry .07 or .08 in sulfur. When this goes

back additional sulfur is picked up, and for this reason it is absolutely necessary to use pig iron as low in sulfur as possible which, of course, is quite expensive.

60 The present invention relates to a novel, cheap, and efficient method of removing this sulfur from the melted cast iron; or at least so much thereof as may be deemed necessary or desirable.

65 In the old Bessemer process melted iron is put into a converter, air blown through the metal until all the silicon, manganese, and carbons are burnt out, the whole reduced to a pure metallic iron, and then sufficient 70 quantities of each were put back to make the grade of steel desired. While my process is somewhat similar, in some respects, to the Bessemer process, at the same time it is radically different therefrom in other respects. 75 In my method melted iron, known as gray or foundry cast iron or malleable iron, is taken from the cupola or furnace and put into a ladle or reservoir either directly or by the aid of other instrumentalities. Air, 80 gas, steam, or some other oxidizing agent is blown through openings in the sides or the bottom of the ladle into and through the molten metal. As the said air, gas or steam or other equivalent comes into contact with 85 the molten metal it oxidizes the manganese creating manganese oxid, which, owing to its affinity therefor, unites with the sulfur to produce slag which rises to the top of the ladle or reservoir where it may be skimmed 90 off, thus reducing the amount of sulfur in the molten metal. During this operation it appears that a small quantity of the manganese unites chemically with the sulfur to form manganese sulfid which also rises to 95 the top of the molten metal, after it is formed, by the agitation produced by the oxidizing agent. So far as can be learned from a study of the process the above appears to be what actually takes place.

100 At the beginning of the process of removing sulfur from cast iron the temperature of the molten metal is substantially the same as the initial temperature of the metal in the Bessemer process. In the latter, however, the temperature increases 105 greatly, due to the oxidation of the carbon and the silicon, by the air blast; while in the present process there is a gradual decrease in the temperature of the molten metal inasmuch as there is no oxidation of the carbon or silicon, or at any rate it is

practically *nil*. This non-oxidation is in turn due to the fact that only an amount of the oxidizing agent is introduced as will cause a slight boiling or ebullition of the 5 molten metal, and I have found that this slight boiling of the metal sufficiently agitates the metal not only to hasten the combination of manganese and manganese oxid with the sulfur but also hastens the separation 10 of the manganese sulfid and the manganese oxid, thus formed, from the molten mass.

In irons low in manganese I put into the ladle ferro manganese to increase the manganese so that there will be more of it to combine with the sulfur. I can also add ferro silicon, carbon or phosphorus by a chamber connected to the air pipe of the ladle to increase my carbon, phosphorus, 20 silicon, or other elements through this chamber. As the air passes through the pipes into the ladle of iron provision is made whereby a siphon effect is created and draws into the molten metal the silicon, 25 phosphorus, manganese, carbons or other elements desired which are introduced to give to the metal the required amount. I also use carbon in different forms blown through this metal to give to the latter 30 some extra heat. I use coke, coal, charcoal, phosphorus or other heat giving material to create and increase the temperature of the molten iron. It is not to be understood that this specific method of adding the elements 35 having the heat giving properties is the only one, as I can introduce them into the bottom of the ladle before pouring the metal into the ladle and obtain substantially the same results. However, the method first 40 described is preferable since it is more accurate. In addition I can also confine all of these elements in a cartridge or retainer and sink them to the bottom of the ladle of metal, the combination being such 45 that it will melt at a lower temperature than the iron. When the elements confined in the cartridge are melted they are given up to the molten metal, part of the manganese being oxidized to form manganese 50 oxid which unites with the sulfur of the molten metal to produce a slag, and the other elements, having heat giving properties, creating more heat for the metal.

My method is to be used in connection 55 with blast furnace work, making pig iron in the usual way, drawing it into a receiver or ladle, treating it as above described and then casting it into pigs. The method is capable of use in all iron or steel foundries 60 in which case the melted metal can flow from the cupola or furnace to this receiver and be treated by this method; or the ladle or receiver can be filled at the cupola and then be transported anywhere desired to be treated.

The process of melting iron chips and casting them into pig iron has always been encountered with serious difficulty on account of the excessive amount of sulfur remaining therein. It is almost invariably 70 found to contain .2 of sulfur which is very high. With this process I can reduce the sulfur of the molten metal made from chips down to .085, which apparently will open up a new field for iron melted from chips 75 and borings thereby enabling one to make pig iron out of this melted chip metal that is so high in sulfur. By experiment it has also been found that 1000 lbs. of iron can be kept alive twenty-five minutes by this 80 process, whereas it would otherwise have set in ten minutes. Iron was also taken containing sulfur .09 and after blowing it fifteen minutes the sulfur was reduced to .06. In another trial beginning with .05 of 85 sulfur air was blown through it for two minutes and test showed it afterward to contain .035 of sulfur and .65 of manganese; after blowing the same batch three minutes longer the test showed sulfur .033 and 90 manganese .52. The slag skimmed off the top of the metal showed sulfur .429 and manganese 2.16. In another test iron was taken containing .074 of sulfur, and after blowing air through it for six minutes the 95 sulfur was reduced to .048. In all these tests just enough air was allowed to pass to keep the metal merely boiling.

Having described my process sufficiently to enable any one skilled in the art to operate the same, what I claim is:

1. The herein described method of removing sulfur from cast iron containing manganese which consists in introducing the molten metal into a ladle or chamber, then oxidizing a part of the manganese and agitating the mass to hasten the combination of manganese and manganese oxid with the sulfur.

2. The herein described method of removing sulfur from cast iron which consists in introducing the molten metal into a ladle or chamber; adding a quantity of manganese; then introducing air to oxidize a part of the manganese and to agitate the mass to hasten the combination of manganese and manganese oxid with the sulfur.

3. The herein described method of removing sulfur from cast iron which consists in introducing the molten metal into a ladle or chamber; adding a quantity of manganese; then introducing an oxidizing agent to oxidize the manganese and to agitate the mass to hasten the combination of manganese oxid and sulfur.

4. The herein described method of removing sulfur from cast iron containing manganese, which consists in introducing the molten cast iron into a ladle or chamber; then introducing an oxidizing agent to oxi-

dize a part of the manganese and to agitate the mass to hasten the combination of manganese and manganese oxid with the sulfur and also to hasten the separation of the manganese sulfid and the manganese oxid thus formed from the mass.

In testimony whereof I affix my signa-

ture in the presence of two subscribing witnesses.

WALTER F. PRINCE.

Witnesses:

J. H. DORCH,  
F. STACKHOUSE, Jr.